

## UNITED STATES PATENT OFFICE

2,512,359

LUBRICANT COMPOSITIONS CONTAINING  
BERYLLIUM CARBOXYLATESJohn F. McGrogan, Philadelphia, Pa., assignor to  
The Atlantic Refining Company, Philadelphia,  
Pa., a corporation of PennsylvaniaNo Drawing. Application October 26, 1946,  
Serial No. 706,054

10 Claims. (Cl. 252—32.7)

1

The present invention relates to lubricants, and particularly to mineral oil lubricants having incorporated therein minor quantities of additive materials adapted to improve lubrication properties, and to inhibit or retard deposition of varnish, lacquer and sludge caused by deterioration of the oil in normal lubrication service.

Commercial petroleum lubricating oils, no matter how highly refined, have a definite tendency to deteriorate under the lubricating conditions encountered in internal combustion engines. High crank case temperatures, and other increasingly severe requirements in engine performance, aggravate the rate of oil deterioration from thermal decomposition and oxidation. Deposits, in the nature of varnish, lacquer and sludge, are products of this deterioration, and in modern engines with close clearances small amounts of these deposits may seriously interfere with proper operation, or may even cause engine seizure. The problems of inhibiting oil deterioration, and of maintaining oil cleanliness during lubrication service, are, therefore, of essential importance, and while the prior art suggests many ways of accomplishing these ends, further improvement is desirable.

It is an object of this invention to provide lubricating oil compositions which are effectively inhibited against the formation of varnish, lacquer and sludge deposits.

I have found that the beryllium salts of carboxylic acids of from 6 to 18 carbon atoms, and particularly of from 12 to 18 carbon atoms, are excellent detergents for all common lubricating oils, and that these compounds as additives in small concentrations minimize deposition of deterioration products, and thereby improve the over-all lubricating properties of the oil. Some of these salts are inherently soluble in petroleum oils in an amount sufficient to provide good detergency action, and those which are less soluble can be readily incorporated in oils with the aid of solubilizing agents, such as aliphatic acids and alcohols, alkyl esters, or other compounds known to have a solubilizing function. The actual amount of salt additive necessary to provide the results intended may vary broadly within a range from about 0.1% to 5.0% by weight of the oil, depending upon the properties of the untreated oil base; and with the more common commercial lubricants, additions of about 0.5% to 2.0% of the beryllium salts have given very satisfactory results.

The beryllium salts which may be employed in accordance with this invention are either the

2

normal or basic salts or mixtures thereof derived from one or a mixture of carboxylic acids. Preference is had for mono- or di-salts of saturated aliphatic carboxylic acids of from 12 to 18 carbon atoms. However, a variety of acids may be employed in the production of the beryllium salts including both the mono- and polycarboxylic acids which are exemplified by enanthic acid, caprylic acid, pelargonic acid, lauric acid, myristic acid, palmitic acid, stearic acid, acids derived by the oxidation of petroleum oils and waxes, adipic acid, pimelic acid, suberic acid, azelaic acid, sebatic acid; succinic acid, and other acids of that series in which one or more of the methylene hydrogens are substituted by unsaturated hydrocarbon residues such as polymers of propylene or butylene having from 8 to 18 carbon atoms; alkylated aryl carboxylic acids including benzoic acid in which one or more of the nuclear hydrogen atoms is substituted by an alkyl or alkenyl group preferably of at least 6 carbon atoms; alkylated polycarboxylic aromatic acids such as phthalic acid in which one or more of the nuclear hydrogen atoms is substituted by an alkyl or alkenyl group of 6 or more carbon atoms; abietic acid, hydrogenated abietic acid, naphthenic acids, and the like.

The beryllium salts of the carboxylic acids may be prepared by reacting a basic beryllium compound, such as beryllium hydroxide or carbonate with the carboxylic acid at elevated temperature, the ratio of hydroxide or carbonate to acid being such as to give either a normal or a basic salt. Alternatively, a soluble beryllium compound such as the chloride, nitrate or sulfate in aqueous solution, may be reacted with an aqueous solution or dispersion of an alkali metal salt of a carboxylic acid to give a water-insoluble beryllium carboxylate. The preparation of the beryllium salts of the carboxylic acids is effected by conventional means, and forms no part of the present invention, therefore, further discussion thereof is not essential.

The beryllium salts of the carboxylic acids may be incorporated in suitable amounts in lubricating oil by simply heating the mixture until solution or dispersion is accomplished, and thereafter cooling the product to ordinary temperatures. When it is desired to increase the anti-corrosion and anti-rust properties of the lubricant, various inhibitors may be added to the oil containing the detergent beryllium carboxylates. The anti-oxidants, anti-corrosion agents, and anti-rust agents may be incorporated in amounts varying from 0.1% to 5% by weight

of the lubricant, 0.5% to 2.0% being preferred. These agents include phenolic and amino compounds such as the long-chain alkylated phenols and polyhydroxy aromatic compounds; aliphatic and aromatic amines; metal salts and amine salts of the acid esters of the acids of phosphorus, and particularly metal salts of the acid esters of a thio-acid of phosphorus such as the zinc salt of cyclohexyl acid thiophosphate; phenol sulfides and metal salts thereof; sulfurized oils and sulfurized esters of carboxylic acids, such as sulfurized aliphatic abietates, sulfurized higher fatty acid esters, sulfurized sperm oil, and the like.

The present invention may be further illustrated by the following examples, which, however, are not to be construed as limiting the scope thereof:

For the detergency test, there is provided a glass test tube within which are vertically and concentrically disposed two sand-blasted open-ended steel tubes. Between the steel tubes is inserted a copper tube of small dimension through which air is delivered to the bottom of the test tube below the end of the inner steel tube. In carrying out the test, the inner steel tube is weighed and then inserted in the testing apparatus. 75 cc. of the oil to be tested is then introduced into the glass test tube and forms a pool covering the lower ends of the steel tubes and the copper tube. The apparatus is then placed in an oil bath and heated to 300° F., air being injected through the copper tube and beneath the surface of the test oil at a rate of 30 liters per hour. After 65 hours heating and blowing, the apparatus is removed from the oil bath and cooled. The inner steel tube is withdrawn, washed with naphtha, and weighed, the increase in weight being attributed to the deposition of sludge. The smaller the weight increase, the more effective the detergent agent in the oil. The results of the tests are tabulated below. The base lubricating oil used was a raffinate fraction of a nitrobenzene selective solvent extracted distillate lubricating stock, such a base oil having an A. P. I. gravity of 31° and a Saybolt Universal viscosity of 175 seconds at 100° F.

| Lubricant                               | Milligrams sludge deposited |
|-----------------------------------------|-----------------------------|
| Base oil                                | 63                          |
| Base oil + 0.5% beryllium mono-stearate | 13                          |
| Base oil + 1.0% beryllium mono-stearate | 3                           |
| Base oil + 2.0% beryllium mono-stearate | 3                           |
| Base oil + 1.0% beryllium di-stearate   | 0                           |
| Base oil + 2.0% beryllium di-stearate   | 1                           |

While, in the above test, a solvent refined lubricating oil was employed as the base, other hydrocarbon oils may be used in lieu thereof, including straight-run lubricating distillates from paraffin base, naphthene base, or mixed base crude oils, acid treated oils, hydrogenated oils, clay treated

oils, deasphaltized residual oils, and synthetic oils produced by the polymerization of olefins or the condensation of olefins or halogenated hydrocarbons with aromatic hydrocarbons.

I claim:

- 5 1. A lubricating oil composition comprising hydrocarbon oil and a beryllium salt of a carboxylic acid containing from 6 to 18 carbon atoms, said salt being present in an amount sufficient to improve the detergency of the oil when used in the lubrication of internal combustion engines.
- 10 2. A lubricating oil composition comprising hydrocarbon oil and from 0.1% to 5% by weight of a beryllium salt of a carboxylic acid containing from 6 to 18 carbon atoms.
- 15 3. A lubricating oil composition comprising hydrocarbon oil and from 0.5% to 2% by weight of a beryllium salt of a carboxylic acid containing from 6 to 18 carbon atoms.
- 20 4. A lubricating oil composition comprising hydrocarbon oil and from 0.1% to 5% by weight of a beryllium salt of a saturated aliphatic carboxylic acid containing from 6 to 18 carbon atoms.
- 25 5. A lubricating oil composition comprising hydrocarbon oil and from 0.5% to 2% by weight of beryllium stearate.
- 30 6. A lubricating oil composition comprising hydrocarbon oil and from 0.5% to 2% by weight of beryllium mono-stearate.
- 35 7. A lubricating oil composition comprising hydrocarbon oil and from 0.5% to 2% by weight of beryllium di-stearate.
- 40 8. A lubricating oil composition comprising hydrocarbon oil, 0.5% to 2% by weight of beryllium stearate, and 0.5% to 2% of a metal salt of an acid ester of an acid of phosphorus.
- 45 9. A lubricating oil composition comprising hydrocarbon oil, 0.5% to 2% by weight of beryllium stearate, 0.5% to 2% of a metal salt of an acid ester of an acid of phosphorus, and 0.5% to 2% of sulfurized ester of a carboxylic acid.
10. A lubricating oil composition comprising hydrocarbon oil, 0.5% to 2% by weight of beryllium stearate, 0.5% to 2% by weight of a metal salt of an acid thiophosphate, and 0.5% to 2% by weight of sulfurized sperm oil.

JOHN F. McGROGAN.

#### REFERENCES CITED

50 The following references are of record in the file of this patent:

#### UNITED STATES PATENTS

| Number    | Name  | Date          |
|-----------|-------|---------------|
| 2,320,392 | White | June 1, 1943  |
| 2,322,307 | Neely | June 22, 1943 |

#### OTHER REFERENCES

- 50 00 The Alkaline Earth and Heavy Metal Soaps, ACS Monograph Series No. 103, 1946, p. 165, by Elliott.